

## UNITED STATES PATENT OFFICE

2,482,423

## COPPER BASE ALLOY

Vincent T. Malcolm, Springfield, Mass., assignor  
to The Chapman Valve Manufacturing Co.,  
Springfield, Mass., a corporation of Massa-  
chusetts

No Drawing. Application March 12, 1947,  
Serial No. 734,222

3 Claims. (Cl. 75—164)

1

This invention relates to the improvement in the alloys and in the manufacturing of alloys wherein copper is the chief constituent.

The principal objects of this invention are to provide an alloy and a method of making the same which will result in an increase in the fluidity and a decrease in the shrinkage or cavity formation tendency in typical alloys containing copper as the chief constituent, with or without tin, zinc, lead, aluminum, or other elements commonly known in the alloying of non-ferrous metals.

It is a further object to provide a modification of grain structure; more particularly it is to provide an elimination of a coarse-loose grain structure, which grain structure results in excessive porosity both microscopically and macroscopically.

The object of the invention is accomplished by the addition of titanium or certain of its alloys or compounds thereof to copper and its various alloys.

Copper and its alloys have been known for a great many years to exhibit substantial casting difficulties due in large part to excessive shrinkage, which has produced flaws and unexpected failures in the hydrostatic test. In one way, this invention includes a method of decreasing shrinkage by shortening the freezing range of the base metal with a resulting increase in the soundness of the casting, and a greater strength in the metal and the homogeneity of the structure, which when hydrostatically tested will be found to be free from any tendency towards leakage due to secondary shrinkage. Furthermore, titanium forms intermetallics in the melt that apparently nucleate grain formation upon cooling of the melt; and as the addition of titanium does not form a solid solution, the macroscopic examination of the metal shows a marked tendency in soundness and homogeneity.

I am aware that copper in combination with titanium has been attempted in the manufacture of non-ferrous alloys but most of the attempts have been found open to objections among which are inability to properly melt, resulting in gas pinholing and segregation of the alloys in the finished product. This deficiency in the finished product, due to the lack of homogeneity and proper holding of the alloys in the copper base,

has resulted in the abandonment of titanium alloys after many failures by other investigators. These failures and many other well known defects inherent to alloys of this class, hitherto known, are obviated by the present invention.

According to this invention, I employ varying amounts of titanium but the addition of 0.10-1.25% has been found to be desirable, preferably an addition approaching 0.50% is desired.

10 In the alloying and manufacturing according to my invention, I proceed as follows:

- 15 A. Since titanium has a high affinity for oxygen, it is necessary to adequately protect titanium so it may be readily wet by the melt.
- 15 B. Titanium has a rather high affinity for both nitrogen and hydrogen so it is absolutely necessary to adequately protect the titanium from contact with these gases.
- 20 C. Titanium has a low density so measures must be provided to insure that the titanium will remain below the surface of the melt during the melting and casting operations.
- 25 D. Titanium has a high melting point so that the addition is preferably made in non-ferrous alloys in the form of a titanium-copper mixture previously cast in accordance with my invention; or if metallic titanium is added, provision must be made to insure that the titanium will be wet by the melt so that a eutectic layer will be formed on the surface of the titanium permitting it to go into solution.

30 The method of melting will be now set forth in detail.

35 *Method A*

- 1. Charge small lumps of metallic titanium, or titanium-copper, of the required alloying amount in the bottom of a crucible or furnace.
- 40 2. Cover the lumps of titanium, or titanium-copper, with one of the following fluxes:

*Flux A.*—Certain preferred amounts of copper oxide, potassium nitrate, borax and ground charcoal.

*Flux B.*—Certain preferred combinations of potassium nitrate, borax and ground charcoal.

- 45 3. Charge the crucible or furnace with copper base metal ingot or any desired combination of copper base non-ferrous alloys.

4. Use a prepared covering consisting of charcoal and borax.

5. Melt to an oxidizing flame and deoxidize with small amounts of phosphorus, usually in the form of copper phosphorus.

6. Careful details must be followed in procedure for time of melting, temperature at which the metal is superheated in the furnace and the resulting pouring temperature of the metal into castings.

*Method B*

All details identical with Method A are used with the exception that .15-.25 metallic silicon is charged with the base metal ingot.

Thus there is produced a metal which has the desirable characteristics set forth herein and overcomes the objections of prior art metals.

The invention may be embodied in other specific forms without departing from the essential characteristics thereof. Hence, the present embodiments are therefore to be considered in all respects merely as being illustrative and not as being restrictive, the scope of the invention being indicated by the appended claims rather than by the foregoing description, and all modifications and variations as fall within the meaning and purview and range of equivalency of the appended claims are therefore intended to be embraced therein.

What it is desired to claim and secure by Letters Patent of the United States is:

1. A method of making a titanium-containing copper alloy consisting in placing metallic titanium in the bottom of a furnace in which the alloy is to be melted, covering said titanium with a flux of potassium nitrate and borax and ground charcoal, charging the furnace with a copper base metal ingot, covering the charged alloy with a mixture of charcoal and borax, melting to an oxidizing flame, deoxidizing with a small amount of phosphorus.

2. A method of producing copper alloy having

fluidity and non-shrinkage characteristics which consists in, placing metallic titanium in the bottom of a crucible, covering the same with a mixture of potassium nitrate, borax and ground charcoal, charging the crucible thereover with copper base metal, covering the same with a mixture of charcoal and borax, melting to an oxidizing flame and de-oxidizing with a small amount of phosphorus, said nitrate, borax and charcoal of the mixture being of such proportions as to act as a flux, and said titanium being from 0.10 to 1.25% of the alloy.

3. A method of producing copper alloy having fluidity and non-shrinkage characteristics which consists in, placing metallic titanium in the bottom of a crucible, covering the same with a mixture of potassium nitrate, borax and ground charcoal, charging the crucible thereover with copper base metal, covering the same with a mixture of charcoal and borax, melting to an oxidizing flame and de-oxidizing with a small amount of phosphorus, said nitrate, borax and charcoal of the mixture being of such proportions as to act as a flux, and said titanium being approximately 0.50% of the alloy.

VINCENT T. MALCOLM.

REFERENCES CITED

The following references are of record in the file of this patent:

UNITED STATES PATENTS

| Number       | Name            | Date          |
|--------------|-----------------|---------------|
| 852,100      | Yunck           | July 3, 1906  |
| 35 1,435,649 | Mihalic         | Nov. 14, 1922 |
| 1,962,606    | Masing et al.   | June 12, 1934 |
| 2,003,889    | Jennison et al. | June 4, 1935  |
| 2,086,604    | Comstock        | July 13, 1937 |
| 40 2,102,238 | Pilling et al.  | Dec. 14, 1937 |
| 2,171,697    | Hensel et al.   | Sept. 5, 1939 |
| 2,195,433    | Silliman        | Apr. 2, 1940  |